

## UNITED STATES PATENT OFFICE

2,367,589

## TANNING

Elbert C. Ladd, Passaic, N. J., assignor to United States Rubber Company, New York, N. Y., a corporation of New Jersey

No Drawing. Application May 13, 1942,  
Serial No. 442,849

3 Claims. (Cl. 8—94.33)

This invention relates to improvements in tanning agents and methods of tanning skins and hides.

Both vegetable and chrome tanning are known methods of producing leather from raw hides. It is also known to use materials known as "Syntans" as auxiliary tanning agents. The Syntans are condensation products of monohydroxyaryl sulfonic acids with aldehydes. It is also known that quinones themselves can be used as tanning agents and such use is described in the literature (for example, J. A. Wilson, "Modern Practice in Leather Manufacturing"—pages 434-435). Simple quinones are not satisfactory tanning agents in that they are relatively insoluble in water and difficult to handle due to irritating effects on the eyes and nasal passages. For these reasons quinone tanning as such has been of only theoretical interest, and according to recognized authorities in the field, it has never been of any commercial importance. I am also aware that both quinone sulfonic acid and sulfonated hydroquinone have been employed as leather tanning agents, but both these materials are less active than benzoquinone itself since it requires from 1½ to 2½ times as much benzoquinone sulfonic acid as of benzoquinone to obtain suitable tanning action.

In an attempt to overcome the disadvantages of the prior methods of tanning, I have produced new leather tanning agents, consisting of 1,4-benzoquinone thiosulfuric acid and its salts. The 1,4-benzoquinone 2-thiosulfuric acid or salt thereof is surprisingly considerably more active as a tanning agent than the corresponding sulfonic acid derivative and is further characterized by being free from the disadvantages possessed by benzoquinone itself.

By the use of my tanning material it is possible to obtain a very high quality leather in a relatively short time. This is due to the fact that my material, unlike vegetable tanning materials, does not exhibit what is known as "case hardening effects," so that it is possible to use relatively concentrated tan liquors without the disadvantages resulting from the use of concentrated vegetable tanning materials. Furthermore, the nature of my tanning material is such as to cause it to penetrate very rapidly into thick hides. This is a particular advantage in the tanning of sole leather.

The optimum pH range for tanning with my material corresponds very closely to the optimum pH range for the tanning with either chrome or vegetable tanning materials. Thus it is pos-

sible to use my improved tanning material in conjunction with other known tanning agents without the necessity of drastic changes in the pH conditions of the tanning liquor.

5 My new tanning agents also appear to increase the effectiveness of tanning assistants or tanning materials such as sulfited lignins. By the use of a combination of my tanning agent and a sulfited lignin, it is possible to obtain a superior grade of leather.

The chemicals may be prepared in several ways, among them being the following:

By reacting quinone with a thiosulfate, thereby obtaining a hydroquinone with an attached 15 thiosulfate radical. This compound may then be suitably oxidized to give the corresponding quinone thiosulfuric acid or salt.

The following examples are given in detail to illustrate the invention, but are not to be understood as limiting thereof:

## Example 1

The potassium salt of 1,4-benzoquinone-2-thiosulfuric acid was prepared according to the method outlined in German Patent No. 175,070. The product, a yellow-orange, crystalline material, is believed to have the formula:



35 A tanning bath was prepared by dissolving 25 grams of the above reaction product in 250 cc. of water at 80° F. The resulting pH of the solution was 2.9. A piece of acetone-dried raw calfskin weighing 53.8 grams was soaked in water 40 until fully saturated, whereupon the wet weight was found to be 240 grams. The skin was then immersed in the tanning solution and the containing vessel was rotated for 3 days. The pH was now 4.6. The skin was removed, and slicked 45 free of excess water, washed in running water for 20 hours and again slicked free of excess water. The weight was now 212 grams. (Shrink temperature was found to be 73° C., compared with 64° C. for the raw hide.) The skin was bleached as follows: 2 grams of sodium borate were dissolved in one liter of water. The skin 50 was shaken in this solution for 15 minutes and then washed in water at 100° F. for one-half hour. The skin was then shaken in a solution of 2 cc. concentrated H<sub>2</sub>SO<sub>4</sub>, in 800 cc. of H<sub>2</sub>O

for 5 minutes, again washed with  $H_2O$  at 100° F. for one-half hour. It was then fat-liquored in a solution of 16 grams of commercial tan oil in 800 cc. of water at 120° F. for 15 minutes. The pH of the fat-liquoring solution was adjusted to 2.7 by addition of  $H_2SO_4$ . The skin was then slicked free of excess oil and allowed to dry at room temperature over night, fat-liquored in a solution of 8 grams of tan oil in 800 cc. of water, slicked and allowed to dry over night. It was then buffed on the flesh side and soaked in water. After having been soaked until thoroughly saturated, it was slicked free of excess fluids and the grain side rubbed with olive oil and set out to dry. After drying over night, it was staked on a knee staker. The resulting product was a well-tanned piece of leather of good quality.

As further evidence of the tanning ability of the above relatively soluble quinone derivative, the following test shows the effect of variations in pH on the tanning efficiency of the quinone derivatives.

Acetone-dried raw calfskin strips weighing approximately 2.5 grams each were used for determination of shrink temperatures. Before being used, they were thoroughly soaked in distilled water to eliminate any "case hardening effect" (i. e., tanning of external portion of the hide which prevents penetration of the tan liquor into the interior). One-half gram of potassium 1,4-benzo-quinone-2-thiosulfate was dissolved in 100 cc. of  $H_2O$ . The resulting solution had a pH of 3.8. A strip of the calfskin was immersed in the solution and the containing vessel was agitated for 24 hours. The final pH of the solution was 5.4. The shrink temperature of the resultant leather was then measured according to the method outlined in the Journal of the American Leather Chemists' Association 36, 681-2 (1941), except that water instead of glycerine was used as the heat transfer medium. The shrink temperature of the treated skin was 78° C. The shrink temperature of the untreated control strip was 66° C. The difference in shrink temperature, namely, an increase of 12° C. is taken as an indication of tannage.

The above test was repeated a number of times with the pH of the liquor adjusted to a different value for each test by adding either 0.1— N HCl or 0.1— N NaOH to the liquor prior to starting the tanning operation. The results are recorded below:

| Grams potassium salt of 1,4-benzoquinone-2-thiosulfuric acid in 100 cc. $H_2O$ | Initial pH | Final pH | Shrink temperature, °C. |
|--------------------------------------------------------------------------------|------------|----------|-------------------------|
| .5                                                                             | 1.9        | 3.2      | 60                      |
| .5                                                                             | 2.0        | 3.4      | 70                      |
| .5                                                                             | 2.3        | 4.1      | 77                      |
| .5                                                                             | 3.4        | 4.4      | 79                      |
| .5                                                                             | 3.8        | 5.4      | 78                      |
| .0 (blank)                                                                     | 5.2        | 6.4      | 66                      |
| .5                                                                             | 8.5        | 6.1      | 68                      |
| .5                                                                             | 8.8        | 6.5      | 63                      |
| .5                                                                             | 9.2        | 6.7      | 61                      |
| .5                                                                             | 10.2       | 7.0      | 60                      |

The data show that our quinone tanning agent increases the shrink temperature of raw hides when used in tanning baths having considerable variations in pH, and that it is particularly effective in baths having pH's in the range 3.5 to 4.5.

A similar series of tests were run, using the sodium salt of 1,4-benzoquinone-2-sulfonic acid, and in all cases the shrink temperature was 6

to 10 degrees lower, thus indicating inferior tanning behavior as compared to my invention.

Another recognized test of tanning ability is to determine the amount of tanning substance combined per 100 grams of hide powder. In such a test, it was found that as much as 18 grams of the 1,4-benzoquinone thiosulfate may be combined with 100 grams of hide powder.

#### Example 2

The tanning agents of my invention may be used in conjunction with other materials which either are tanning agents in themselves or have an auxiliary action. For example, a tanning bath

15 containing the compound prepared in Example 1 together with a commercial lignosulfonic acid sold under the name of "Super-Spruce" was prepared by dissolving 6.25 grams of the potassium salt of 1,4-benzoquinone-2-thiosulfuric acid and 25 grams of Super-Spruce in 250 grams of water. The resulting pH was noted to be 2.6. A piece of acetone-dried raw calfskin weighing 51.7 grams was soaked in water until saturated then slicked free of excess  $H_2O$  (wet weight 226 grams). It was then placed in the tan liquor and agitated for 72 hours. The skin was then worked up in the same way as described in Example 1. The result was a piece of well-tanned leather of good quality.

20 It is to be understood that the tanning materials do not have to be isolated from the solutions in which they are prepared. One may also prepare a tanning liquor, for example, by oxidizing any suitably substituted benzene thiosulfuric acid or salt thereof in an aqueous medium to obtain an aqueous solution of a 1,4-quinone thiosulfuric acid or salt thereof. Such solutions can be used directly as the tanning liquors. Various oxidizing agents may be used in the preparation of these derivatives. For example, one may use a chromium compound such as sodium dichromate or chromic anhydride as the oxidizing agent. The tan liquor prepared by such a reaction will contain both the desired benzoquinone derivative and the chromium salt, the latter being in a suitable state to produce tanning effects. Such a solution, therefore, will provide a tanning action due to both a chromium salt and the soluble quinone derivative.

25 The invention is not limited to the methods of preparation used in the illustration. Other methods of preparing the quinone derivatives are known and may be used. For example, para-aminophenol-ortho-thiosulfuric acid, or a salt thereof, can be oxidized in an aqueous medium to produce a solution of the quinone derivative, which solution is an effective tanning liquor.

30 It is to be understood that the invention is not to be limited to the compounds given in the examples. Although it appears that the tanning action is due primarily to the quinone thiosulfuric acid, or a salt thereof, other products may be formed during the oxidation, which may aid in the tanning action. For example, quinones are known to form complexes with hydroquinones. Furthermore, controlled oxidation of a hydroquinone (or controlled reduction of a quinone) may lead to complex derivatives. One type of such complexes is known as a quinhydron. It is possible that such complexes are formed by methods herein described and that they may contribute to the tanning action. Such derivatives may be formed by methods used in preparing the quinone derivatives and are understood to be within the broad scope of my

invention. For this reason the present products are generally defined as oxidation products of substituted benzene thiosulfuric acids, and their salts, which substituted acids and salts have the property of being oxidized to quinone thiosulfuric acids, or their salts. The more common substituents in the aryl nucleus, which on oxidation provide the final quinone nucleus, include dihydroxy, amino, di-amino, etc., radicals.

Having thus described my invention, what I claim and desire to protect by Letters Patent is:

1. A method of tanning skins or hides which comprises immersing the same in an acid bath containing a tanning agent comprising an oxidation product of 1,4 substituted benzene 2-thiosulfuric acids, and their salts, which substituted acids and salts have the property of being oxidizable to the corresponding quinone thiosulfuric acid, and their salts, respectively.

2. A method of tanning skins or hides which comprises immersing the same in an acid bath

containing a tanning agent comprising a compound having the general formula



10 where X is a radical selected from the class consisting of hydrogen, and an alkali-metal.

15 3. A method of tanning skins or hides which comprises immersing the same in an acid bath containing a tanning agent comprising a quinonoid oxidation product of a compound of the class consisting of amino benzene 2-thiosulfuric acids and hydroxy benzene thiosulfuric acids, and their salts, which compound is capable of being oxidized to para-quinone ortho-thiosulfuric acid.

20 ELBERT C. LADD.